

## UNITED STATES PATENT OFFICE

2,055,417

PROCESS FOR LOWERING THE POUR  
POINT OF MINERAL OILSFranz Rudolf Moser, Amsterdam, Netherlands,  
assignor to Shell Development Company, San  
Francisco, Calif., a corporation of DelawareNo Drawing. Application August 30, 1935, Serial  
No. 38,576. In the Netherlands October 3, 1934

20 Claims.

(CL. 87—9)

This invention relates to a process for manufacturing hydrocarbon oils with a low pour point or cold test or equivalent inspection test, such as lubricating oils, Diesel fuels, fuel oils, etc., and 5 to a hydrocarbon oil composition having a low pour point.

In accordance with the present invention the pour point, cold test, or equivalent inspection test of such hydrocarbon oils is lowered by the 10 addition to such oils of soaps of the tetravalent form of a metal from the titanium subgroup of Group IV and higher carboxylic acids. Thus, it was found that soaps containing any of the 15 metals of the titanium subgroup, such as zirconium, hafnium and thorium may be employed, but I have obtained best results with titanic soaps, and prefer them to the other soaps.

The titanium soaps can, for example, be prepared by reacting the metallic chloride with the 20 anhydrous carboxylic acid, as described by L. W. Ryan and W. W. Plechner in Ind. Eng. Chem., 26, (1934) p. 909.

The carboxylic acids which are employed in producing the soaps used according to the present invention should contain between ten and 25 thirty, or even more carbon atoms, may be mono- or poly-basic, and may be either saturated or not. Thus, I have found fatty acids, such as stearic acid, palmitic acid, oleic acid, linoleic acid, behenic acid, cerotic acid to be particularly suitable. 30 Other examples of carboxylic acids which I have found to be suitable for reaction with the metal chloride to form the desired soaps are: naphthenic acids, such as tetradeca-, hexadeca- and nonadeca-naphthenic acids, and mixtures of 35 naphthenic acids as obtained by extracting petroleum with sodium hydroxide solutions; colophonic acids, such as abietic acid and pimaric acid; oxy-acids, such as ricinoleic acid; oxidation products of paraffin wax.

Besides the neutral salts of the tetravalent metals of the titanium subgroup, also basic salts 40 may be used as pour point reducers. Thus, although the theoretical  $TiO_2$  content of titanic tetrastearate is about 6.75%, I have obtained good results when using titanic soaps containing around 9% and even higher amount of  $TiO_2$ . The  $TiO_2$  content should, however, preferably be not over about 13.5%. I have, moreover, 45 found that the best results are obtained when the soap contains four acyl side chains.

The pour point reducing agents according to the present invention are generally more active than the soaps of bivalent and trivalent metals, 50 such as zinc oleate and aluminum stearate, which

have heretofore been used for this purpose. They have the additional advantage of a comparatively smaller ash content.

In treating hydrocarbon oils with the soaps according to my invention, a small quantity, usually between 0.02% and 1.0% is added to a wax-containing oil, preferably but not necessarily at a temperature at which the wax is wholly or substantially liquid or dissolved in the oil. It should be noted that my invention is not, however, restricted to the use of the aforesaid quantities, since the quantity of soap to be employed in any case will depend upon the decrease in the pour point which it is desired to effect, upon the quantity and nature of the wax present in the oil, and upon the viscosity of the oil. Thus it was found that pour point reducers have a comparatively greater effect on paraffinic oils of low viscosity, and in the case of fuel oils or Diesel fuels amounts as low as 0.01% or lower 20 may often be effective. My invention may, however, be applied also to the treatment of the more viscous hydrocarbon oils, such as cylinder oils and other lubricating oils.

The effect of certain of my soaps on hydrocarbon oils is illustrated in the following examples:

## Example I

A Pennsylvania turbine oil had a pour point of  $-4^{\circ} C$ . Upon adding 0.05% of titanic stearate, prepared according to the method of Ryan and Plechner, Ind. Eng. Chem. 26 (1934) p. 909, the pour point was found to be below  $-20^{\circ} C$ .

## Example II

An extra heavy neutral oil derived from Pennsylvania and Mid-Continent crudes had a pour point of  $10^{\circ} F$ . Upon adding 0.5% of titanium stearate (containing 8%  $TiO_2$ ) the pour point was reduced to  $0^{\circ} F$ . The addition of 1.0% of titanium stearate reduced the pour point to  $-5^{\circ} F$ .

I claim as my invention:

1. A low pour point mineral oil composition comprising wax-containing mineral oil and a small quantity of a soap of the tetravalent form of a metal of the titanium subgroup of group IV and a carboxylic acid containing more than nine carbon atoms.

2. The composition according to claim 1 in which the quantity of the soap is between 0.01% and 1.0% of the composition.

3. A low pour point mineral oil composition comprising wax-containing mineral oil and a small quantity of a soap of the tetravalent form of a metal selected from the group consisting

- of titanium, hafnium and thorium, and a carboxylic acid containing more than nine carbon atoms.
4. A low pour point mineral oil composition comprising wax-containing mineral oil and a small quantity of a titanic soap of a carboxylic acid containing more than nine carbon atoms.
5. The composition according to claim 4 in which the quantity of the soap is between 0.01% and 1.0% of the composition.
6. A low pour point mineral oil composition comprising wax-containing mineral oil and a small quantity of a thoric soap of a carboxylic acid containing more than nine carbon atoms.
- 15 7. A low pour point mineral oil composition comprising wax-containing mineral oil and a small quantity of a hafnic soap of a carboxylic acid containing more than nine carbon atoms.
8. The composition according to claim 1 in which the soap contains four acyl side chains.
9. The composition according to claim 3 in which the soap contains four acyl side chains.
10. The method of reducing the pour point of wax-containing mineral oils which comprises adding thereto a small quantity of a soap of the tetravalent form of a metal of the titanium subgroup of Group IV and a carboxylic acid containing more than nine carbon atoms.
- 15 11. The method according to claim 10 in which the quantity of the soap is between 0.01% and 1.0% of the wax-bearing mineral oil.
12. A low pour point mineral oil composition comprising wax-containing mineral oil and a small quantity of a titanium tetrastearate soap of a carboxylic acid containing more than nine carbon atoms.
- 20 13. The method of reducing the pour point of wax-containing mineral oils which comprises adding thereto a small quantity of a soap of the tetravalent form of a metal from the group consisting of titanium, hafnium and thorium, and a carboxylic acid containing more than nine carbon atoms.
14. The method of reducing the pour point of wax-containing mineral oils which comprises adding thereto a small quantity of a titanic soap of a carboxylic acid containing more than nine carbon atoms.
- 15 15. The method according to claim 14 in which the quantity of the soap is between 0.01% and 1.0% of the wax-bearing mineral oil.
16. The method of reducing the pour point of wax-containing mineral oils which comprises adding thereto a small quantity of a thoric soap of a carboxylic acid containing more than nine carbon atoms.
- 20 17. The method of reducing the pour point of wax-containing mineral oils which comprises adding thereto a small quantity of a hafnic soap of a carboxylic acid containing more than nine carbon atoms.
18. The method according to claim 12 in which the soap contains four acyl side chains.
19. The method according to claim 13 in which the soap contains four acyl side chains.
- 25 20. The method of reducing the pour point of wax-containing mineral oils which comprises adding thereto a small quantity of titanium tetrastearate.

FRANZ RUDOLF MOSER. 35